

June 15, 1926.

1,589,023

W. E. TRENT

PROCESS FOR CRACKING COAL AND OIL

Filed Sept. 27, 1924



Inventor  
Walter E. Trent

By Charles M. Thomas

Attorney

Patented June 15, 1926.

1,589,023

# UNITED STATES PATENT OFFICE.

WALTER EDWIN TRENT, OF WASHINGTON, DISTRICT OF COLUMBIA

REISSUED

## PROCESS FOR CRACKING COAL AND OIL.

Application filed September 27, 1924. Serial No. 740,385.

The invention relates to improvements in processes for the production of purified solid fuels in conjunction with the production of liquid motor fuels.

carry out the operation with the greatest possible heat efficiency and economy and further to produce definite quality forms of both solid and liquid fuels.

5 The purified solid fuel is made by amalgamating finely pulverized coal with an oil residuum obtained by first evaporating the lighter boiling fractions from a crude or fuel oil.

60 The heat utilization is practiced by using;—

10 The heat for evaporating these lighter fractions is generated by the isothermal compression of the evaporated vapors and then imparting this heat to the original oil through the medium of a heat exchanger.

65 A boiler and steam actuated compressor, the pressure steam to actuate the oil vapor compressor, the exhaust steam from the compressor to be utilized to heat the water used in the amalgamator box. The boiler stack gases are used to heat the amalgam baking apparatus. The heat generated by oil vapor compression is to be utilized to vaporize

15 It is necessary to use a residuum with a high percentage of asphalt or carbon so that the resulting amalgam of the coal particles and residuum, when baked or carbonized, will provide the binder for making hard, 70

75 strong fuel masses.

the original charging stock oil; to utilize the heat in the vaporized oil fractions leaving the baking apparatus by subjecting same while in vapor form to cracking pressure and temperature, the utilization of the sensible heat of the oil residuum to make amalgam.

20 It is not the intention to use a residuum

80 that will make hard and strong fuel masses in a green state by merely briquetting or shaping and then cooling. They are only

25 to be so after baking and carbonizing and the residuum is to be such that from about 40 to 80% of same will vaporize under the baking or carbonizing treatment. These vaporized fractions are conducted to and

85

30 mixed with the evaporated fractions derived from the original charging stock that enters the heat exchanger and simultaneously compressed, then cooled and liquefied by circulating through the heat exchanger in tubes surrounding by the oil to be evaporated.

90

35 The positive displacement compression of these vapors is to develop the combination of pressure and temperature that causes the maximum degree of cracking of the vapors 95 into lighter boiling fractions and the heat of compression so generated is to be transferred to and cause the vaporization of the original oil. The compressed vapors constitute, when condensed, a pressure distillate from 100 which is to be extracted and refined the desired fractions of liquid motor fuel by any of the existing methods, and the remaining fractions are to be added to the residuum from the heat exchanger or to the original 105 charging stock to undergo the treatment cycle a second time.

105

40 The invention particularly relates to a process broadly described in my Patent No. 1,420,165 relating to the purification of coals 110 by amalgamation with oils obtained by the distillation of the product and aims to

115

Referring now more particularly to the drawings wherein like reference characters indicate corresponding parts, the numeral 1 designates an amalgamator in which finely pulverized coal of say 100 meshes to the linear inch is introduced, preferably in water suspension, through the feeding line. This amalgamator contains a series of agitators for thoroughly agitating the material therein. To this amalgamator I also introduce liquid hydrocarbon residuum oils, which oils are delivered hot after having had the lighter fractions removed by evaporation.

120 Exhaust steam is introduced to this amalgamator which was first generated in a boiler plant 3 having the boiler tubes 4 and a boiler 5 therein, and then expanded in oil vapor compressor. The boiler is fired in any well known manner, the steam being introduced

to the amalgamator in a way to be herein-after described.

The material undergoing amalgamation in the amalgamator is such as described in my patent aforesaid, and when discharged from the amalgamator consists of plastic mixtures of coal and oil of a consistency resembling putty, usually in the form of spherical bodies of desired diameters. These bodies, or 10 masses, are largely free of water and detached ash. They are deposited on the screen 6 so as to be separated from water and ash, and this screen carries them to a hopper 7, there to be formed or moulded 15 into desired shapes and conveyed through an elongated baking oven 8, which is heated by smoke stack gases from the steam boiler. The purpose for baking or carbonizing the formed fuel masses is to make them hard and 20 strong so they may be transported, and handled, to make them smokeless under combustion, or substantially so, to remove the oils vaporized at the temperatures employed and to convert them into light boil- 25 ing motor fuel fractions.

Adverting now to the steam boiler, it will be seen that the steam from this boiler discharges through a line 10 to a compressor cylinder 11, being exhausted from this cylinder through a line 12 into the amalgamator 1. Hot boiler gases from the boiler also discharge through the line 13 into the baking oven 8 to supply the necessary heat to this oven to bake or carbonize the material passing therethrough. Suitable valves are provided for controlling the passage of the heating gases through these lines.

It will be observed that the steam from the boiler 5 first passes to the steam compressor cylinder 11. This steam is there utilized to operate a compressor 14 employed for the purpose of subjecting hydrocarbon vapors to a high degree of compression to crack said vapors. The steam exhausting 40 from the power compressor cylinder 11 then passes to the amalgamator. In the process described crude oil, or other charging stock, is fed from a tank 15 passing therefrom through a line 16 from where a portion of the oil can pass through a line 17 to the jacket 18 of the vapor compressing cylinder to control the temperature of compression in said cylinder while the major part of the oil supply passes through the line 19 to a 50 space 20 in the elongated heat exchanger 21. That part of the oil passing through the jacket of the vapor compressing cylinder also enters the space 20 through the line 22 in a somewhat preheated condition. In the 55 space 20 of the heat exchanger there are a plurality of tubes 23 receiving the compressed vapors, by means of which the heat of the cracked vapors is indirectly imparted to the charging stock in a manner now to be 60 described.

A substantial part of the liquid charging stock entering the space 20 is vaporized, the vapors passing from this space through the line 25 to the compressor 14 where said vapors are subjected to an exceedingly high 70 stage of compression, this exothermic compression raising the temperature of the vapors to a cracking condition of temperature and pressure so that they undergo substantial conversion in said compressor. The 75 cracked vapors from the compressor while at a cracking temperature, discharge through the line 27 into the tubes 23 passing through the interior of the heat exchanger. These hot vapors serve to vaporize substantial portions of the incoming charging stock to provide the vapors that are to enter the compressor 14. The vapors by being robbed of their heat largely condense in the tubes 23 and the condensate flows out through the 80 line 28 into the receiver 29 employed for collecting the converted products. The space 20 of the heat interchanger is preferably maintained under a vacuum so as to lower the vaporizing point of the incoming charg- 85 ing stock. The unvaporized oil from this chamber consisting of large quantities of heavy oils, tar, pitch, carbon, etc., is continuously withdrawn through the line 30 and collected in a receiver 31 from where it is 90 conveyed by the line 32 directly to the amalgamator 1. It will also be understood that the amalgamated product passing through the baking oven 8 is subjected to a temperature of say 550° F., to 1,000° F., and that 95 the volatiles contained in both the coal and the oil constituting this amalgamated product are vaporized either in part or to any degree desired depending on temperature, time of treatment and type of solid product 100 wanted, these vapors passing through the line 33 to the line 25 for passage on to the compressor 26 to undergo cracking by reason of the high temperature and pressure they attain due to the high compression of these 110 vapors.

As an illustration of an operation, coal of a bituminous character, preferably of a fineness of 100 meshes per linear inch, is introduced in water suspension to the amalgamator, and there mixed with a liquid hydrocarbon residue containing substantial quantities of carbon base. The quantity of hydrocarbon material used is approximately in the proportion of one part hydrocarbon 115 material to five parts coal by weight. The amalgamated material is deposited on the screen 6 and after being formed into masses of uniform size, is then introduced to the baking oven 8 which is heated by furnace 120 gases passing through the line 13. This oven is maintained at a temperature of say 650° to 700° F., causing a vaporization of the lighter volatiles contained in the oil 125 and the coal, leaving the heavier substances 130

therein which retain a substantially solid state in the carbonized masses discharged from the oven on the receiver adjacent the outlet thereof. The vapors generated in the oven pass on to the vapor line 25 for passage to the converting compressor 26 together with other vapors produced from crude oil and in a manner now to be described. During this operation crude oil 10 from the tank 15 is passing through the space 20 of the heat interchanger and this oil is heated therein to a temperature of say 590° F. to 600° F. When a plant is being placed in operation, the oil may be heated 15 by steam from the boiler passing through the tubes 23. After the plant is in operation the oil is then heated by heat absorbed from cracked vapors. A substantial part of this oil, however, is vaporized and these 20 vapors of a temperature of say 500° F. to 600° F. pass through the line 25 into the compressor 26 where they are subjected to a high degree of compression of say 100 pounds per square inch, which raises the 25 temperature of the vapors to approximately from 700° to 850° F., this temperature being controlled by the passage of oil through the jacket 18 of the compressor. The compressor is operated by the compressor cylinder 30 11 receiving steam from the line 10 which communicates with the boiler 5. After the vapors are heated to a cracking temperature in the compressor 14 they then pass through the line 27 into the tubes 23 of the heat ex- 35 changer 26. Here the vapors heat the charging stock and are themselves largely condensed, constituting converted low boiling point oils. Such oils flow through the line 28 into the receiver 29. The unvaporized 40 oil in the chamber 20 is withdrawn through the residual line 30 by a pump, or the like, depositing into the tank 31 from where it is continuously introduced to the amalgamator 1 for the purposes hereinbefore 45 described.

From the foregoing description of the process, it will be seen that I produce solid clean smokeless fuels and liquid motor fuels, that the manufacture of the solid fuel contributes to the yield of liquid fuel, that the production of motor fuel contributes a liquid residuum necessary to the successful manufacture of the solid fuel, that waste or by-product heat incidental to the production 55 of each product is successfully utilized in the production of the other.

Having thus described my invention, what I claim is:

1. A process for manufacturing a carbonized solid fuel and converting low boiling point oils by heat generated at a single source, consisting in utilizing a portion of said heat for subjecting oils to cracking conditions of temperature and pressure, and 60 in employing by-product heat for carboniz- 65

ing comminuted fuels to produce a carbonized residue.

2. A process for manufacturing carbonized fuels of a solid nature and converting hydrocarbon oils, consisting in developing 70 heat energy by combustion of a fuel at a single source, in utilizing said heat for subjecting hydrocarbon vapors to a heat compression sufficient to crack the same, in employing waste gases for heating the solid 75 fuel to remove volatiles therefrom and produce a carbonized residue.

3. A process for manufacturing solid carbonaceous fuels and converting hydrocarbon oils by heat energy developed at a single 80 source, consisting in utilizing a part of the energy for compressing oil vapors to subject said vapors to cracking temperatures and pressures, in mixing hydrocarbon oil with pulverized coal while in water suspension, 85 and in utilizing a portion of the energy for heating said water during the agitation of the materials.

4. A process for manufacturing solid carbonaceous fuels and converting hydrocarbon 90 oils by heat energy developed at a single source, consisting in utilizing a part of the energy for compressing oil vapors to subject said vapors to cracking temperatures and pressures, in mixing hydrocarbon oil with 95 pulverized coal while in water suspension, in utilizing a portion of the energy for heating said water during the agitation of the materials, and in also utilizing waste heat of combustion from said single source for removing oils from the agglomerated material producing a carbonized mass.

5. A process for manufacturing solid carbonaceous fuels and converting hydrocarbon oils by heat energy developed at a single 100 source, consisting in utilizing a part of the energy for compressing oil vapors to subject said vapors to cracking temperatures and pressures, in mixing hydrocarbon oil with pulverized coal while in water suspension, 105 in utilizing a portion of the energy for heating said water during the agitation of the materials, in also utilizing waste heat of combustion from said single source for removing oils from the agglomerated material producing a carbonized mass, and in subjecting said removed oils in the form of vapor to said cracking conditions of temperature and pressure.

6. A system of treating hydrocarbon materials, consisting in generating heat at a single source by the combustion of fuel, in utilizing a portion of the heat to convert hydrocarbon oils by subjecting oil vapors to cracking conditions of temperature and pressure in a compressor utilizing said energy, in passing said vapors through a preheater to vaporize charging stock being admitted to the compressor, in withdrawing unvaporized oil from said preheater, in introducing said 110 115 120 125 130

oil to an amalgamator, in mixing said oil in the amalgamator with coal in water suspension, in utilizing a part of said heat produced at a single source for heating the water in 5 said amalgamator, in discharging the agglomerates from said amalgamator, in distilling said agglomerates by heated gases generated at said single source, and in introducing the vapors and gases obtained from 10 said agglomerates to said compressor for conversion.

7. A process for amalgamating coals and cracking hydrocarbon oils, consisting in mixing hydrocarbon residue with finely pulverized coal and water, in introducing charging stock to a heat interchanger where a portion thereof is vaporized, in subjecting said vapors to a high compression by a heat energy operating a compressor engine, in 15 passing the compressed vapors through the heat interchanger to vaporize portions of the charging stock, in collecting the low boiling point 20 oils thus produced, in withdrawing residual oil from said heat interchanger and utilizing the same for agglomeration with the coal, in maintaining the water during such 25 agglomeration in a heated condition by waste heat from said compression, in passing the agglomerates to an oven, in vaporizing oil fractions from said agglomerates in said oven, and in passing said fractions to said compressor for conversion therein.

ing the water during such agglomeration in a heated condition by waste heat from said compression:

8. A process for amalgamating coals and cracking hydrocarbon oils, consisting in mixing hydrocarbon residue with finely pulverized coal and water, in introducing charging stock to a heat interchanger where a portion thereof is vaporized, in subjecting said vapors to a high compression by a heat energy operating a compressor engine, in passing the compressed vapors through the heat interchanger to vaporize portions of the charging stock, in collecting the low boiling point 40 oils thus produced, in withdrawing residual oil from said heat interchanger and utilizing the same for agglomeration with the coal, in maintaining the water during such 45 agglomeration in a heated condition by waste heat from said compression, in passing the agglomerates to an oven, in vaporizing oil fractions from said agglomerates in said oven, and in passing said fractions to said 50 compressor for conversion therein.

In testimony whereof I affix my signature.  
WALTER EDWIN TRENT.